

April 24, 1951

C. L. FAUST

2,550,544

METHOD OF ANODICALLY POLISHING ALUMINUM

Filed Nov. 14, 1947

3 Sheets-Sheet 1



INVENTOR  
CHARLES L. FAUST

THE SIGN OF CHARLES FAUST HHS

April 24, 1951

C. L. FAUST

2,550,544

METHOD OF ANODICALLY POLISHING ALUMINUM

Filed Nov. 14, 1947

3 Sheets-Sheet 2



*Inventor*  
CHARLES L. FAUST

*Fig. 4* *The Firm of Charles Faust* *Fig. 5*

April 24, 1951

C. L. FAUST

2,550,544

METHOD OF ANODICALLY POLISHING ALUMINUM

Filed Nov. 14, 1947

3 Sheets-Sheet 3



INVENTOR  
CHARLES L. FAUST

Fig. 7 The Firm of Charles L. Faust Attn:

## UNITED STATES PATENT OFFICE

2,550,544

METHOD OF ANODICALLY POLISHING  
ALUMINUM

Charles L. Faust, Columbus, Ohio, assignor, by  
mesne assignments, to Battelle Development  
Corporation, Columbus, Ohio, a corporation of  
Delaware

Application November 14, 1947, Serial No. 786,092

3 Claims. (Cl. 204—140.5)

1

This invention relates to an electrolyte comprising an aqueous solution of sulfuric, phosphoric and chromic acids and to methods of anodically polishing aluminum and aluminum alloys in said electrolyte.

In the anodic electropolishing of aluminum on a commercial scale, it is desirable to operate at a relatively low voltage, for instance, from 7 to 15 volts; to operate at a relatively low current density, for instance, from 60 to 200 amperes per square foot; and to operate with the same bath for a maximum length of time or, at least, with only such adjustments in the composition of said bath as can be carried out without interruption of polishing.

In my copending application, Serial No. 569,641 filed December 23, 1944 (now abandoned) and entitled "Electrolyte for and Method of Anodically Polishing Metals," of which the present application is a continuation-in-part, I have disclosed electrolytes adapted for polishing aluminum comprising an aqueous solution of sulfuric, phosphoric and chromic acids. However, although operative, the compositions of this copending application will not always electropolish aluminum at the commercially most desirable voltages or current densities or for such length of time (without reconditioning) as is most desirable for commercial purposes.

It is therefore an important object of the present invention to provide electrolytes for and methods of anodically electropolishing aluminum operative at low voltages, low current densities and for long periods of time.

Other and further objects and features of the present invention will become apparent from the following description, drawings, and appended claims.

The electrolytes according to the present invention comprise essentially from 4 to 45% (by weight) of sulfuric acid (100%  $H_2SO_4$ ), from 40 to 80% of phosphoric acid (100%  $H_3PO_4$ ), from 0.2% or preferably 0.4% to saturation of chromic acid (100%  $CrO_3$ ), and from 0 to 6% of dissolved metals (aluminum, or aluminum and trivalent chromium), the balance being essentially water. The total acid concentration ranges from 50 to 95%. Such baths are operative to electropolish aluminum at a voltage of 15 volts or less and at a current density ranging from 25 to 950 amperes per square foot, the current density varying according to the viscosities of the baths, as will be disclosed in greater detail hereinbelow. Preferably, the baths are operated at a current density of from 60 to 150

or 200 amperes per square foot, a temperature of from 160 to 200° F., a viscosity of from 9 to 13 centipoises (at the operating temperature of, say, 180° F.) and a voltage of from 7 to 15 volts. Suitable agitation of the bath is effected, the exact amount and type depending on the shape and size of the articles being polished, the number of articles being polished, the spacing of the articles and of the cathodes, the size and shape of the tank, and like factors.

A specific bath according to the present invention comprises 4.7% sulfuric acid, 75% phosphoric acid, and 6.5% chromic acid, the balance being essentially water together with not more than 4.5% of dissolved aluminum, or of dissolved aluminum and trivalent chromium. This bath is preferably operated at a current density of from 60 to 150 amperes per square foot, a temperature of from 175 to 185° F. (with some variation depending on dissolved aluminum, or aluminum and trivalent chromium content, as described hereinbelow), a viscosity of from 10 to about 11.5 centipoises, and a voltage of from 7 to 12 volts.

The practical significance of the features disclosed hereinabove will be apparent from the following discussion.

Figure 1 is a graph showing the permissible maximum concentrations of dissolved aluminum for electropolishing at not more than 15 volts in baths having a relatively constant sulfuric acid plus phosphoric acid concentration, and having the sulfuric acid concentrations shown in the abscissae.

Figure 2 shows the relationship between specific gravity and viscosity of a polishing bath containing 4.7% sulfuric acid, 75% phosphoric acid, and 6.5% chromic acid with respect to the dissolved aluminum content.

Figure 3 is a chart showing the temperatures required for the production of a mirror finish on aluminum at a current density of 100 amp./sq. ft. and a voltage of 12 to 15 volts with respect to variations in the dissolved aluminum content, using the same bath as in Figure 2.

Figure 4 is a graph illustrating how the temperature must be increased and the specific gravity lowered in a bath containing 4.7% sulfuric acid, 75% phosphoric acid, and 6.5% chromic acid to maintain a constant viscosity despite increase in the dissolved aluminum content.

Figure 5 is a graph illustrating the increase in voltage at various temperatures when using a bath containing 5% sulfuric acid, 80% phos-

phoric acid, and water containing varying amounts of dissolved aluminum.

Figure 6 shows the operating characteristics of a bath containing 15% sulfuric acid and 63% phosphoric acid with varying amounts of dissolved aluminum at an operating temperature of 200° F.

Figure 7 is a graph showing the viscosity in centipoises required for electropolishing at a voltage of 12.5 volts at various current densities using a bath containing 4.7% sulfuric acid, 75% phosphoric acid, and 6.5% chromic acid.

Figure 8 is a graph showing how the bath used in Figure 5 must be operated at higher temperatures as the dissolved aluminum content is increased.

Figure 9 shows the operating characteristics of a bath comprising 45% sulfuric acid and 45% phosphoric acid and containing varying amounts of dissolved aluminum.

Figs. 3, 6 and 9 show certain combinations of current density, voltage and temperature operative for the production of a mirror polish on aluminum in baths containing various amounts of dissolved aluminum. The three baths of Figs. 3, 6 and 9 are aqueous solutions of phosphoric and sulfuric acids containing various amounts of dissolved aluminum but devoid of chromic acid. The latter acid has been omitted from these baths for the reason that the chromic acid, except by providing a source of trivalent chromium, does not affect the electropolishing operation one way or another during the time the electropolishing current is kept flowing. The function of the chromic acid is that of protecting the mirror finish after the flow of electropolishing current has been terminated, when the aluminum is subject to etching attack by a bath devoid of chromic acid.

In Fig. 3 are shown the temperatures required for the production of a mirror finish on aluminum when it is desired to electropolish at 100 amp./sq. ft. and to keep the voltage in the range of 12 volts to 15 volts while the dissolved aluminum content varies. The figures within the circles show the voltage required to establish a current density of 100 amps./sq. ft. at the indicated dissolved aluminum content and at the temperature designated.

As shown by Fig. 3, aluminum can be electropolished to a mirror finish in a bath containing 5% sulfuric acid, and 80% phosphoric acid at a dissolved aluminum content ranging from 0 to 4.5% without any need for raising the current density above 100 amperes per square foot or for raising the voltage above 15 volts. Further, it is not necessary to raise the temperature to a value of 200° F. until a dissolved aluminum content of 3.0% has been reached.

Fig. 6 shows the operating characteristics of a bath containing 15% sulfuric acid and 63% phosphoric acid, the balance being essentially water together with various amounts of dissolved aluminum. In the case of this bath, all operating data relate to a temperature of 200° F., since electropolishing cannot be carried out below this temperature at relatively low current densities or voltages. Further, the data relate to contents of dissolved aluminum not greater than 1.5%, for the reason that at higher contents of dissolved aluminum electropolishing cannot be carried out at relatively low current densities or voltages. Each circle in the chart of Fig. 6 represents a current density operative at the indicated content of dissolved aluminum,

and the operating voltage for that particular current density has been inserted within each circle. Unlike Fig. 3, Fig. 6 shows not only the minimum current density operative at a particular content of dissolved aluminum, but various other and higher operative current densities, together with the voltages required to maintain all these operative current densities.

Fig. 9 relates to the operating characteristics of a bath comprising 45% sulfuric acid and 45% phosphoric acid, the balance being essentially water together with various amounts of dissolved aluminum. All the data of Fig. 9 refer to an operating temperature of 200° F. and a dissolved aluminum content of not more than 1.5%, for the reason that electropolishing cannot be effected with this bath at relatively low current densities or voltages at temperatures of less than 200° F. or at contents of dissolved aluminum in excess of 1.5%. Otherwise, the chart of Fig. 9 makes the same showing as the chart of Fig. 6.

Thus, as shown by the data in the graphs of Figs. 3, 6 and 9, a low sulfuric acid content (as compared to the phosphoric acid content) makes possible electropolishing at higher dissolved aluminum contents; at lower voltages; at lower current densities; and, at dissolved aluminum contents of 2.0 or less, at lower temperatures.

Reference is also made to Fig. 1 showing the permissible maximum concentration of dissolved aluminum for electropolishing at not more than 15 volts in baths containing sulfuric and phosphoric acids in various ratios but having approximately the same total sulfuric-phosphoric acid concentration. As shown, quite high concentrations of dissolved aluminum permit electropolishing at not more than 15 volts in baths containing less than 10% sulfuric acid, while no electropolishing at 15 volts is possible in baths containing 65% or more sulfuric acid.

The above noted adverse effect of increasing the sulfuric acid content (at the expense of the phosphoric acid content) obtains normally at relatively high total acid concentrations (at about 85% total acid concentration or higher). At lower total acid concentrations, a higher proportion of sulfuric acid will not interfere with electropolishing at from 10 to 15 volts. For instance, a bath containing 32.5% sulfuric acid, 42.6% phosphoric acid and 1.6% chromic acid, the balance being essentially water, will satisfactorily polish aluminum at 10 to 15 volts.

While, at higher total acid concentrations, best results are obtained with relatively low concentrations of sulfuric acid, the presence of these relatively small amounts of sulfuric acid is nevertheless necessary at all total acid concentrations for best results.

The operating characteristics of baths devoid of sulfuric acid are indicated hereinbelow. Baths containing from 50 to 85% phosphoric acid and, optionally, chromic acid, but no sulfuric acid, will electropolish aluminum but with some pitting of the aluminum or at undesirably high voltages, current densities or temperatures or at various undesirably narrow ranges of voltage, current density or temperature. For instance, for electropolishing in baths containing, respectively, 50% and 70% phosphoric acid, at 100 amperes per square foot, there are required, respectively, voltages of 21 and 35 volts. In the case of a bath containing 75% phosphoric acid and 1.2% dissolved aluminum, the balance being essentially water, aluminum can be electropolished at current densities of from 100 to 250

amperes per square foot at 180° F. with a voltage ranging from 16 to 40 volts. At other temperatures, a different current density range is required. In the case of baths containing 50% phosphoric acid and 1.2% dissolved aluminum, the balance being essentially water, electropolishing is effected at 180° F., a current density of from 150 to 550 amperes per square foot, and a voltage of from 10 to 24 volts. Best electropolishing, however, is effected at a current density of from 450 to 550 amperes per square foot, and a voltage of from 19 to 24 volts. A bath consisting of 80% phosphoric acid and 20% water performs essentially similarly to the bath containing 75% phosphoric acid.

The operating characteristics of baths containing sulfuric acid in amounts of less than 4% are given as follows. Addition, for instance, of 2% sulfuric acid to a bath containing 85% phosphoric acid causes some luster, but full brilliance is not obtained. However, increasing the sulfuric acid content to 5% makes possible a brilliant mirror-like finish.

The benefit to be derived from the presence of sulfuric acid is further demonstrated by electropolishing tests in a bath containing 80% phosphoric acid and 7% chromic acid, the balance being essentially water. This bath is the equivalent of the preferred bath containing essentially 4.7% sulfuric acid, 75% phosphoric acid and 6.5% chromic acid, apart from the sulfuric acid. In other words, adding sulfuric acid to a bath containing 80% phosphoric acid and 7% chromic acid will yield the preferred bath. In such a bath containing 80% phosphoric acid and 7% chromic acid, electropolishing takes place at a current density of from 100 to 250 amperes per square foot, a voltage of from 5 to 28 volts, and a temperature of 180° F. However, the aluminum, although lustrous, is pitted. At 30 to 50 amperes per square foot, the luster is uneven and pitting is also evident. Attempts to electropolish at lower temperatures in the bath containing 80% phosphoric acid and 7% chromic acid either lead to anodizing or require excessive voltages.

With respect to the chromic acid of the acid content of the bath of the present invention, it should be noted that, as pointed out hereinabove, the chromic acid is added to prevent chemical attack of the aluminum after termination of electropolishing and while the polished aluminum is still wetted with the polishing bath. At least 0.4% chromic acid should be incorporated with the bath for best results. Chromic acid may be present in any amount from 0.2% to saturation. The presence of chromic acid does not immediately affect the electropolishing. However, any trivalent chromium formed as a result of the reduction of chromic acid has the same effect as dissolved aluminum. In other words, the presence of trivalent chromium will lower the permissible concentration of dissolved aluminum so that the life of the bath is correspondingly shortened.

The formation of trivalent chromium is caused by cathodic reduction of the chromic acid. This action can be prevented by using porous ceramic media around the cathode. These media form a closed cup in which 85% phosphoric acid is used as a catholyte to carry the current to the cathodes placed therein. The porous medium around the cathodes decreases the amount of chromic acid entering the reducing environment. Whatever chromic acid does enter the catholyte is reduced to trivalent chromium which remains in the

cathode chamber where it does not act to shorten the life of the electropolishing bath. Thus, there is no significant formation of trivalent chromium outside of the porous cathode cups and the electropolishing life is, accordingly, not shortened by such formation. The use of porous cups for preventing, or greatly retarding, such cathodic reduction is well known in the field of electrolysis, and details for effecting the result desired may be varied in accordance with such knowledge.

The general operating conditions for the baths of the present invention have been disclosed hereinabove. More specific details are given hereinbelow.

Reference is made to the graph of Figure 7. This graph shows the viscosity (in centipoises) required for electropolishing at constant voltage (12.5 volts) at various current densities for a bath initially containing 4.5% sulfuric acid, 75% phosphoric acid, and 6.5% chromic acid, the balance being essentially water. As shown, the viscosity must be lowered as higher current densities are applied, if the voltage is to be maintained at a constant value. Such lowering of viscosity may be effected by dilution with water, by operation at a higher temperature, or by both methods, as will be discussed in greater detail hereinbelow.

In the preceding paragraph it has been shown that the initial viscosity must be regulated if higher current densities are to be applied without the use of an excessively high voltage. However, as the dissolved aluminum content (and also the trivalent chromium content) of a bath increases when the bath is used for electropolishing aluminum, this increased dissolved metal content causes an increase both in the specific gravity and in the viscosity of the bath. Reference is made to Figure 2 as showing the specific gravity and viscosity at various dissolved aluminum contents. At these increased specific gravities and viscosities, higher voltages must be applied to maintain the current density, and the operating temperature must also be raised. Figure 5 shows graphically the increase in voltage at various temperatures in a bath containing 5% sulfuric acid, 80% phosphoric acid and water, at various contents of dissolved aluminum. Reference is also made to Fig. 8 as showing how the operating temperature must be raised as the dissolved aluminum content is increased.

Fig. 4 shows how the temperature must be increased and the specific gravity lowered (by the addition of water), in a bath containing 4.5% sulfuric acid, 75% phosphoric acid and 6.5% chromic acid, the balance being essentially water, if the viscosity is to be maintained constant in spite of an increased dissolved aluminum content due to continued operation.

In general, there is an upper limit of aluminum concentration, which is reached in the use of the baths herein disclosed and which is dependent upon the sulfuric acid/phosphoric acid ratio and the total acid concentration.

It is thus apparent that, while the baths of the present invention are operative at current densities of from 25 to 950 amperes per square foot, the desired initial low voltage conditions are not obtained except by regulation of the initial viscosity of the bath. Further, if the desired low voltage is to be maintained throughout the life of the bath, the initial viscosity should be maintained at its original value, or within the limits indicated, as by addition of water to the bath and/or increasing the operating temperature, or both.

The methods of this application are operative to electropolish aluminum and aluminum alloys containing at least 90% aluminum but not over 1% silicon. Examples of such metals are commercially pure aluminum (99.4 to 99.0% aluminum, 1.0 to 0.6% iron, and small amounts of silicon and copper); commercially pure aluminum containing 1.2% manganese; an alloy of commercially pure aluminum containing 4% copper, 0.5% manganese and 0.5% magnesium; an aluminum alloy containing 1.9% copper, 0.6% magnesium, 1.0% silicon and 96.5% aluminum; an alloy containing 2.5% magnesium and 0.25% chromium, the balance being essentially aluminum; and an alloy containing 4.4% copper, 0.8% silicon, 0.8% manganese, 0.4% magnesium and the balance essentially aluminum.

Many details of composition and procedure may be varied within a wide range without departing from the principles of this invention and it is therefore not my purpose to limit the patent granted on this invention otherwise than necessitated by the scope of the appended claims.

I claim as my invention:

1. A method of electropolishing aluminum and aluminum alloys containing at least 90% aluminum and not over 1% of silicon, which comprises making the aluminum the anode in a composition initially comprising essentially from 4 to 45% by weight of sulfuric acid, from 40 to 80% by weight of phosphoric acid, and from 0.2% by weight to saturation of chromic acid, maintaining a total amount of dissolved aluminum and trivalent chromium during continued operation not in excess of 6%, the balance being essentially water, and the total acid concentration being from 50 to 95% by weight of said composition, and passing a current through said composition at a temperature of from 160° to 200° F., an anodic current density of from 25 to 950 amperes per square foot and a voltage not in excess of 15 volts.

2. A method of electropolishing aluminum and aluminum alloys containing at least 90% aluminum and not over 1% of silicon, which comprises making said aluminum the anode in a composition initially comprising essentially from 4 to 45% by weight of sulfuric acid, from 40 to 80% by weight of phosphoric acid, and from 0.2% by weight to saturation of chromic acid, main-

taining an amount of dissolved aluminum such that the total amount of dissolved aluminum and trivalent chromium during continued operation is not in excess of 6% by weight, the balance being essentially water and the total acid concentration being from 50 to 95% by weight, and passing a current through said electrolyte at an anodic current density of from 60 to 150 amperes per square foot, at temperature of from 160° to 190° F., and a voltage of from 7 to 15 volts, and maintaining said composition during said electropolishing at a viscosity of from 9 to 13 centipoises as measured at operating temperature.

3. A method of electropolishing aluminum and aluminum alloys containing at least 90% aluminum and not over 1% of silicon, which comprises making said aluminum the anode in a composition initially comprising essentially from 4 to 45% by weight of sulfuric acid, from 40 to 80% by weight of phosphoric acid, and from 0.2% by weight to saturation of chromic acid, maintaining an amount of dissolved aluminum such that the total amount of dissolved aluminum and trivalent chromium during continued operation is not in excess of 6% by weight, the balance being essentially water and the total acid concentration being from 50 to 95% by weight, and passing a current through said electrolyte at an anodic current density of from 60 to 150 amperes per square foot, at a temperature of from 160° to 190° F., and a voltage of from 7 to 15 volts, and adding water as necessary to said composition to maintain said composition during said electropolishing at a viscosity of from 9 to 13 centipoises as measured at operating temperature.

CHARLES L. FAUST.

#### REFERENCES CITED

The following references are of record in the file of this patent:

#### UNITED STATES PATENTS

| Number    | Name  | Date          |
|-----------|-------|---------------|
| 2,040,617 | Mason | May 12, 1936  |
| 2,338,321 | Faust | Jan. 4, 1944  |
| 2,366,714 | Faust | Jan. 9, 1945  |
| 2,429,676 | Faust | Oct. 28, 1947 |

#### OTHER REFERENCES

"Proceedings of American Electroplaters Society," June 1946, pp. 50, 51, 67.